

## UNITED STATES PATENT OFFICE

2,352,822

## PHOTOGRAPHIC COATING

John Dessauer, Irondequoit, N. Y., assignor to  
The Haloid Company, Rochester, N. Y., a corporation of New York

No Drawing. Application February 2, 1942,  
Serial No. 429,280

2 Claims. (Cl. 95—7)

This invention relates to a photographic light sensitive coating and has for its object to afford an improved coating particularly adapted for photographic enlarging paper, contact printing paper, and reflex copy paper.

One purpose of the invention is to afford a coating requiring less time than heretofore for properly completing a given exposure on enlarging paper and which possesses a high degree of sensitivity when exposed to light within the general region of the spectrum comprehended between 4400 and 5200 angstroms, the spectral wave light region within which the light most generally used for photographic exposures has a highly satisfactory actinic value.

Another purpose of the invention is to afford a coating with extreme sensitivity in the spectral region within which the more efficient results are had for most color separation work.

A further object of the invention is to afford a coating containing a dye that is not sensitive to the pH value of an emulsion and does not lose sensitivity in the presence of halogen and free silver ions but is stable and influenced very little by such factors so that instead of impairing the stability or keeping qualities of the emulsion as is the case with dyes heretofore used, it has the further advantage of improving the character and lasting qualities of the emulsion.

An additional object of the invention is to improve the results obtained with as well as the quality of reflex copy paper which is exposed in a contact printer with the coated side out and the subject to be copied is placed face down against the coating, with a light source arranged to direct light through the coated light sensitive paper on to the subject to be copied, the light being absorbed by the printed portions and reflected back on to the light sensitive coating where it strikes an unprinted or white portion.

In the production of reflex copy paper, the best results have heretofore been obtained by using a sensitizing dye in the emulsion and in addition a desensitizer, the function of which is to desensitize the emulsion so as to slow down its exposure speed and make possible the use of such a paper in subdued daylight, but a desensitizer has a practical disadvantage since its desensitizing action on the coating continues and renders it unfit for successful use after it has been stored for a length of time, and it is an additional purpose of the invention to afford a reflex copy paper that will attain equally good and better photographic results without the use of a desensitizer, thus preventing deterioration of the

coating after storage and maintaining its efficiency regardless of its age.

It is a further purpose of the invention to provide a coating sensitized with a dye that gives the best range for color sensitivity, preferably between 4400 and 5200 angstroms, thus affording a more selective color control, and which also greatly reduces the exposure time required within this desirable region of the spectrum.

Another object of the invention is to afford a coating for photographic papers containing a sensitizing dye that gives a sufficiently high speed in the dye-sensitized region to enable using a slow emulsion or one which initially requires a long exposure time, thus enabling the use of an emulsion that is low in silver content.

A further purpose of the invention is to afford an enlarging paper coating containing a sensitizing dye that gives to the coating a much faster exposure speed than heretofore in the dye-sensitized region in relation to the speed of the initial emulsion.

An additional object of the invention is to afford a chloride emulsion coating having an exposure speed as fast as that of a bromide emulsion while retaining the desirable advantages of the chloride emulsion.

The purposes of the invention may be accomplished with a silver chloride emulsion, or a silver bromo-chloride emulsion containing approximately one-third to one-half bromide and two-thirds to one-half chloride, by adding the dye solution to the emulsion either during the mixing process at any time after the silver halide is formed, or shortly before the emulsion is coated on the paper or support. The dye solution may consist of one part of dye to one thousand or two thousand parts of solvent, either water or alcohol, and satisfactory results have been obtained by adding 0.1 to 0.2 gram of such a dye solution to approximately forty pounds of emulsion.

Dyes which have been found satisfactory in obtaining the results as stated above are phosphine or chrysanthilin nitrate, the formula for which is  $C_{12}H_{12}N_3 + NO_3$ , acridine orange or tetramethyl diamino acridin chlorhydrat, the formula for which is  $C_{17}H_{20}N_3Cl + ZnCl_2$ , and acriflavine or diamino methyl acridinumchlorid-chlorhydrat, the formula for which is  $C_{14}H_{14}N_3Cl + HCl$ . These are acridine dyes, each containing two benzene rings united by carbon and nitrogen respectively, and experiments already conducted indicate that the invention can be successfully carried out with any of the acridine dyes.

These dyes give a highly satisfactory degree of sensitivity in the region of the spectrum between 4400 and 5200 angstroms with an extremely fast exposure speed in relation to the initial speed of the emulsion in the color region to which it is naturally sensitive. It has been ascertained that where a silver chlorine emulsion had an initial speed of approximately thirty-five seconds, the dyes mentioned will increase the speed to approximately five seconds in the dye-sensitized region of the spectrum. With these dyes, an exposure speed can be obtained with a chloride or bromo-chloride emulsion as fast as the speeds attainable with bromide emulsions, while retaining the desirable characteristics of the chloride emulsion, which gives a better photographic result and is easier to prepare and handle than a bromide emulsion coating.

The dyes herein disclosed enable the manufacture of coatings that are particularly adapted to color photography work by giving a fast exposure speed within the general spectral region from 4400 to 5200 angstroms. Spectrograms made from coatings sensitized with acriflavin, phosphine, and acridine orange show high speed sensitivity at 4400 to 4800 angstroms, 4600 to 5200 angstroms, and 4400 to 5200 angstroms respectively, all within the spectral region that is best adapted to color separation work.

Most printing and exposing of photographic paper is done with Mazda light which has increased actinic radiation toward the longer wave lengths and the dyes herein disclosed sensitize the emulsion to color within a spectral region that is well adapted and extremely efficient when working with Mazda light.

The most satisfactory results have been obtained with silver chloride emulsion, although it is possible to use the dyes with some degree of success with silver chloro-bromide emulsions containing not more than one-half bromide.

The dyes disclosed, owing to their exposure speed, permit the use of a slow emulsion and hence one of low silver content, thus reducing cost particularly in the case of contact papers. The dyes disclosed are stable as against the pH value of an emulsion or the halogen and free silver ions which it contains and have no deteriorating influence on the coating, the efficiency of which is not reduced or impaired with age, but on the contrary, the quality of the coating appears to be improved by the dye, so that no fogging is present and the photographic results are excellent.

When used for reflex copy paper, the use of a desensitizer is unnecessary and the keeping quality of the paper is considerably better than when a desensitizer is employed while the speed

in relation to the natural emulsion is quite sufficient for practical and successful results.

The dyes disclosed are of low cost, simple to produce, easily obtainable commercially, and they can be incorporated readily in the emulsion owing to their chemical nature. They impart to the coating of enlarging paper a faster speed relatively to the natural emulsion than dyes heretofore used for this purpose, and help to give the necessary keeping quality to the emulsion that is required for practical requirements. The results obtained are substantially better both as to the image obtained and the stability of the coating than enlarging papers heretofore obtainable, and when used for contact papers, an emulsion with a lower silver content than heretofore can be employed without affecting the resulting image. Thus the ease of handling and other advantages that characterize a chloride emulsion are had while retaining the speed of a bromide emulsion but without any of the undesirable characteristics of the latter.

Other advantages and results will develop from use of the dyes set forth in a light sensitive silver haloid coating, and this application is intended to cover such adaptations of the invention as may come within the purposes of the improvement and the scope of the following claims.

I claim:

30 1. A photographic coating which can be exposed for printing in subdued daylight under Mazda light and contains one of the group of emulsions consisting of silver chloride emulsion, and silver bromo-chloride emulsion containing approximately one-third to one-half bromide and two-thirds to one-half chloride, and an acridine dye which enhances the keeping power of the emulsion and imparts to the coating high speed sensitivity confined within the spectral region between not less than 4400 angstroms and not more than 5200 angstroms.

2. A photographic coating which can be exposed for printing in subdued daylight under Mazda light and contains one of the group of emulsions consisting of silver chloride emulsion, and silver bromo-chloride emulsion containing approximately one-third to one-half bromide and two-thirds to one-half chloride, and one of the group of dyes consisting of chrysanthin nitrate, tetramethyl diamino acridin chlorhydrat, and diamino methyl acridiniumchlorid-chlorhydrat, which enhances the keeping power of the emulsion and imparts to the coating high speed sensitivity confined within the spectral region between not less than 4400 angstroms and not more than 5200 angstroms.

JOHN DESSAUER.